

## 1

3,323,882

**COMPOSITE GRID WIRE FOR ELECTRON TUBES**  
 Henry J. Albert, Colts Neck, N.J., assignor to Engelhard Industries, Inc., Newark, N.J., a corporation of Delaware  
 No Drawing. Filed Dec. 6, 1966, Ser. No. 599,364  
 3 Claims. (Cl. 29—193)

### ABSTRACT OF THE DISCLOSURE

The present invention deals with a composite emission inhibiting grid wire for electron tubes which resists embrittlement at high operating temperatures, which has high tensile strength and maintains a resistance against grain-growth and creep at elevated temperatures, and which is composed of a core of interfused wires of a 50/50 molybdenum-rhenium alloy with the core being coated with titanium.

### Background of the invention

In electron tubes employing hot electron emissive cathodes of the activated type, e.g. thoriated cathodes, in conjunction with grids of a refractory material, e.g. tungsten, tantalum and molybdenum, which must be essentially free of activation material, it has been found that the grids suffer from contamination by the activation material and lose stability unless protected by an electron emission inhibiting material. Generally, the grids are coated with an electron emission inhibiting material comprising a coating of platinum, gold or titanium.

Such coated grids, while effectively inhibiting electron emission, have a tendency to become embrittled when employed for long periods at the elevated operating temperatures of the tubes, the embrittlement being caused by the grain-growth of the grid metal with a consequent short stress-rupture time which limits the useful life of the grid.

### Summary of the invention

In accordance with the invention, it has been found that a grid wire having a core composed of about 50/50 molybdenum-rhenium alloy with the core being coated with a layer of titanium provides an effective emission inhibiting grid structure which is characterized by high tensile strength and resistance against breakage by creep and grain-growth at elevated temperatures when the core metal is in a fibrous form of interfused wires.

### Description of the preferred embodiments

In providing the composite grid wire of the invention, a substantially heavy-walled titanium tube is prepared. For example, the tube may have a wall thickness of about 0.065" with an O.D. of about 0.540" and a length of about 6.0".

Also, a suitable length of wire having a diameter of about 0.20" and composed of about 50/50 molybdenum-rhenium alloy is provided. The term "about 50/50 molybdenum-rhenium alloy" includes an alloy composition of 48%—52% molybdenum and 52%—48% rhenium by weight percent. The wire is cut into lengths of about

## 2

6.0" to substantially correspond with the length of the titanium tube. Both the titanium tube and the molybdenum-rhenium wires are thoroughly cleaned by known procedure to remove surface contaminants. Between about 150 to about 200 of the wires are inserted into the titanium tube and the composite rod is reduced by cold swaging initially to about 50% reduction which is possible due to the elimination of the voids between the wires. Thereafter, the composite rod is reduced to wire by alternately annealing and cold drawing with the average reduction between anneals ranging from about 25% to about 37.5% reduction. The annealing is accomplished by heating the composite in vacuum at about 1000° C., for example, between about 1200° C. to 1600° C. for from 2 to 3 hours, and the wire is thusly drawn to about 0.032" diameter. During the working of the composite wire, the core wires became interfused into a mass having a fibrous grain structure such that the fibrous grains are elongated along the length of the core and the core is bonded directly to the coating layer.

The mechanical properties of the resultant composite wire is shown in the following table:

TABLE I

|                                     | Tensile Strength, p.s.i.g. U.T.S. | Elongation, Percent in 2" |
|-------------------------------------|-----------------------------------|---------------------------|
| Cold Worked Condition, 0.032" dia.  | 170,000                           | 3                         |
| Vac. Annealed Condition (1,200° C.) | 138,000                           | 3                         |

It will be seen that the elongation of the composite wire is substantially constant in both the cold worked and annealed condition, which is a result of the core composed of the fibrous interfused wires.

When the composite wire of the invention is employed as a grid in electron tubes operating at high temperatures, there is practically no embrittlement of the grid because the transformation of the plurality of core wires by interfusion into a fibrous mass of elongated grains resists embrittlement at high operating temperatures by inhibiting grain-growth of the core grains.

Consequently, the composite grid wire of the invention is characterized by a long useful life during operation of the electron tubes.

What is claimed is:

1. A composite emission inhibiting grid wire for electron tubes, comprising a core in the form of a mass of interfused wires in fibrous form composed of an alloy of 48% to 52% molybdenum and 52% to 48% rhenium, and a coating of titanium bonded directly to the core.
2. A composite grid wire according to claim 1, wherein in the core is composed of a 50/50 molybdenum rhenium alloy.
3. A composite grid wire according to claim 1, wherein in the composite wire is characterized by a substantially constant elongation both in the cold-worked and annealed conditions.

No references cited.

HYLAND BIZOT, Primary Examiner.